

April 8, 1952

2,592,368

E. C. YACKEL  
GELATINE SILVER HALIDE EMULSION LAYER CONTAINING  
A DIHYDROXY DIPHENYL TANNING DEVELOPING AGENT

Filed Nov. 4, 1947

FIG. 1.



FIG. 2.



FIG. 3.



EDWARD C. YACKEL  
INVENTOR

*Edward C. Yackel*  
BY *R. Frank Smith*  
ATTORNEYS

## UNITED STATES PATENT OFFICE

2,592,368

GELATINE SILVER HALIDE EMULSION  
LAYER CONTAINING A DIHYDROXY  
DIPHENYL TANNING DEVELOPING  
AGENTEdward C. Yackel, Rochester, N. Y., assignor to  
Eastman Kodak Company, Rochester, N. Y., a  
corporation of New Jersey

Application November 4, 1947, Serial No. 783,912

4 Claims. (Cl. 95—6)

1

This invention relates to light-sensitive photographic materials and particularly to improved types of sensitized materials suitable for making images in tanned colloid vehicle.

In the sensitized photographic tracing cloth at present available a silver halide emulsion is coated on a subbed tracing cloth which has generally been waterproofed. This material sometimes has the disadvantage that the processed cloth shows a bad tendency to curl which interferes with its every-day use and with filing of the finished drawing. Another disadvantage is that erasures and corrections on the processed sheet are difficult because of the presence of gelatin. In another type of tracing cloth in which bichromated gelatin is used the photographic speed of the material is extremely low and the unexposed or unprocessed material has poor keeping properties.

I have found that it is possible to incorporate a tanning developing agent into a photographic emulsion on a support such as tracing cloth and after exposure and development to form relief images by washing the unexposed emulsion away with water. However, if a soluble tanning developing agent such as pyrocatechol or hydroquinone is used, because of solubility, vapor pressure, etc., the developing agent does not remain in the emulsion layer during long periods of keeping. Instead, it wanders throughout the gelatin and waterproofing layer of a material such as tracing cloth and from one piece of material to another when the two are in close contact. This wandering of the developing agent results in undesirable stain, poor developability, etc. However, if a substantially water-insoluble tanning developing agent is used in the emulsion layer the objections to a more soluble type of developing agent are overcome. In addition, when emulsion layers are compounded with the substantially water-insoluble tanning developing agents according to my invention such emulsion layers are eminently suitable for use in a process of the type described and claimed in Yutzy and Yackel U. S. patent application, Serial No. 783,914 filed concurrently herewith.

It is therefore an object of the present invention to provide light-sensitive photographic emulsion layers containing substantially water-insoluble tanning developing agents. A further object is to provide a sensitized tracing cloth having improved properties. Other objects will appear from the following description of my invention.

These objects are accomplished in part by incorporating a substantially water-insoluble tan-

2

ning developing agent in a light-sensitive photographic emulsion layer, and further, by coating such an emulsion layer on a tracing cloth or other support and after exposure and development in an alkali solution, treating the element with warm water to wash away the undeveloped silver halide with its vehicle. This leaves a tanned colloid relief image on the tracing cloth or other support and provides an image carrying material which is substantially free from curl and on which erasures or corrections can be made and which has good keeping properties.

In the accompanying drawings, the three figures are enlarged cross-sectional views of the tracing cloth at various stages in my process.

According to my invention a light-sensitive silver salt emulsion layer containing a substantially water insoluble tanning developing agent is prepared. According to my method of using such an emulsion layer it is coated on a support such as tracing cloth, a cellulose ester film base, glass, or paper. Fine-grain gelatino-silver bromide emulsions are preferably used but silver chloride or other silver halide emulsions may be used in gelatin or other vehicles such as polyvinyl alcohol, which can be differentially tanned with tanning developing agents.

The developing agent may be any substantially water-insoluble developing agent which tans the gelatin or other carrier for the silver halide, upon development in an alkaline solution. Examples of tanning developing agents specially useful because of their non-wandering characteristics, high rate of development, high tanning efficiency, and solubility in the preferred range, are those having a solubility of from about .005 to 1.0 gram per hundred cc. of a phosphate citric acid buffer solution of pH 5.0 prepared from a 1.5 per cent solution of sodium dihydrogen phosphate and sufficient citric acid to bring the pH to 5.0. The preferred developing agent has the solubility of from about .01 to 0.2 gram per hundred cc. of buffer solution. Developing agents following within the above classification are, for example, 3,4-dihydroxy diphenyl; 2,5-dihydroxy diphenyl; 2,3-dihydroxy diphenyl; and 5,6,7,8-tetrahydro napthohydroquinone. Compounds like 2-hydroxy-5-amino-diphenyl or 3,4-diaminodiphenyl are not especially useful because of their poor stability characteristics or failure to differentially tan the emulsion vehicle.

Here and in the appended claims wherein it is stated that the developing agents are substantially water-insoluble this is defined as meaning

tanning developing agents having solubility within the above range of buffer solution.

Here and in the appended claims wherein it is stated that the emulsion vehicle is substantially unhardened this is defined as meaning not harder than would be the case with gelatin containing 0.25 ounce of formaldehyde (40 per cent solution diluted 1 to 3 with water) per pound, when freshly coated, or 0.1 ounce of the solution per pound for a sample aged three to six months. Emulsion layers appreciably harder are not very satisfactory for use in my process or that of the above coperenting application.

In general, when utilizing the usual type of photographic gelatin useful results are obtained without addition of hardener to the emulsion. In case the gelatin in use has poor physical properties then a small amount of hardener such as formaldehyde may be used.

The emulsion layer prepared as above is exposed in the usual manner under a line drawing and is "developed" by immersion in an aqueous solution of an alkali such as sodium or potassium carbonate, an alkali metal hydroxide such as sodium hydroxide, potassium hydroxide, or ammonium hydroxide, or an amine. The addition to the alkaline solution, of other materials, is also helpful in obtaining a satisfactory relief image. For example, the addition of sodium hydroxide to a sodium carbonate solution improves the sensitometric characteristics of the material as well as the relief properties. The addition of reducing agents such as ascorbic acid, hydrazine hydrochloride, sodium sulfite, in small quantities, sodium bicarbonate and urea, are also advantageous.

After development of the exposed material in the alkaline solution the element is washed with warm water to remove the unexposed and undeveloped colloid and silver halide and then dried. By "warm" water I mean water at a temperature of about 90° F. to 100° F. or higher.

My invention will be further understood by reference to the following examples which are illustrative only.

#### Example I

A method of making an emulsion suitable for use in making a tracing cloth or in the process of the Yutzy and Yackel application Serial No. 783,914, is as follows: Solutions are made of (A) 25 grams of gelatin in 1 liter water at 40° C., (B) 100 grams silver nitrate in 500 cc. water at 20° C. and (C) 35 grams of sodium chloride in 500 cc. of water. Solutions B and C are simultaneously run into Solution A at a uniform rate while stirring the latter over a period of about 10 minutes; Solution B preferably not being allowed to run in faster than C. Thereafter, 150 grams of gelatin in 1500 cc. of water at 40° C. are added. The emulsion is then adjusted to pH of 5.0. If desired, the emulsion may then be chilled, set, and washed in the usual manner. It is then remelted and 25 grams of 3,4-dihydroxy diphenyl dissolved in 250 cc. of methyl alcohol is slowly added to the above emulsion with stirring. As a result the developing agent becomes dispersed in the emulsion in minute crystals. Preparatory to coating an emulsion layer, in case a gelatin having poor physical properties has been used, 2 cc. of 10% formaldehyde may be added and this composition is coated on a prepared tracing cloth support over an area of about 500 square feet and dried. The dried product is exposed to a suitable negative and developed in a 4 percent sodium carbonate

solution. The developed element is then washed with water at 35° C. to remove the unexposed, undeveloped and untanned emulsion, is then rinsed and dried. A positive relief image in gelatin is thus obtained with no gelatin remaining in the unexposed area. Erasures and redrawing of lines were as satisfactory on the print as on the uncoated tracing cloth. Curl was greatly diminished and was approximately equivalent to that of the uncoated tracing cloth, after having been processed through the same baths.

#### Example II

15 Another emulsion suitable for use in my invention is made from the following solutions—(A) 25 grams gelatin in 1 liter water at 40° C.; (B) 100 grams silver nitrate dissolved in 500 cc. water at 20° C.; (C) 72 grams potassium bromide in 500 cc. water at 20° C. Solutions B and C are simultaneously run into Solution A with stirring and afterwards a solution of 200 grams gelatin in 2 liter water at 40° C. is added. A suitable surface-active agent may then be added and the pH adjusted to 5.0. Thereafter a solution of 25 grams of 4-phenyl catechol in 250 cc. of methyl alcohol is added with stirring. Preparatory to coating the emulsion on a support as tracing cloth, a small quantity of hardener may be added as in Example I following which the emulsion is coated over an area of about 300 square feet.

20 The concentration of developing agent in the emulsion is dependent in part on the result desired but can be of the order of 350 grams per kg. of silver nitrate, converted to silver halide, used in making the emulsion, to obtain good density, or about 250 grams per kg. of silver nitrate to obtain adequate density and an emulsion having optimum keeping properties.

25 In the accompanying drawings, I have shown a typical tracing cloth at various stages in my process. As shown in Fig. 1, a support 10 of sized tracing cloth is coated with a gelatino-silver halide emulsion 11 containing a substantially water insoluble tanning developing agent. 30 This material is exposed and developed by immersion in an alkaline solution to form images of silver and hardened gelatin as shown at 12 in Fig. 2. The remaining unhardened gelatin and silver halide 13 in Fig. 2 is then washed off by treatment of the tracing cloth with warm water to leave images 14 of hardened gelatin on the support 10 as shown in Fig. 3.

35 I am aware that the incorporation of organic developing agents in emulsions to form self-developing emulsions is well known and that the use of hardening developers in solution to form hardened gelatin images for use in the production of relief images, is also known. However, I am not aware that substantially water-insoluble hardening developing agents of the type specified above have been incorporated in light-sensitive silver salt emulsions and the resulting emulsions used to form tanned images.

40 My invention having been described, I would have it understood that the disclosure herein is by way of example and included in the invention are all modifications and equivalents falling within the scope of the appended claims.

45 What I claim is:

46 1. A photographic emulsion layer comprising a substantially unhardened gelatin vehicle and dispersed in said vehicle a silver halide and a tanning developing agent of the class consisting of 2,3-dihydroxy diphenyl, 2,5-dihydroxy diphenyl, and 3,4-dihydroxy diphenyl.

2. A photographic emulsion layer comprising gelatin, silver halide, and 2,3-dihydroxy diphenyl.  
 3. A photographic emulsion layer comprising gelatin, silver halide, and 2,5-dihydroxy diphenyl.  
 4. A photographic emulsion layer comprising gelatin, silver halide, and 3,4-dihydroxy diphenyl.

EDWARD C. YACKEL.

## REFERENCES CITED

The following references are of record in the 10 file of this patent:

## UNITED STATES PATENTS

| Number    | Name        | Date          | Number    |
|-----------|-------------|---------------|-----------|
| 742,405   | Eichengrun  | Oct. 27, 1903 | 15 23,251 |
| 1,102,028 | Fischer     | June 30, 1914 | 581,479   |
| 1,472,048 | Christensen | Oct. 30, 1923 |           |

| Name              | Date          |
|-------------------|---------------|
| Troland           | Apr. 25, 1925 |
| Procoudine-Gorsky | Apr. 16, 1929 |
| Procoudine-Gorsky | July 7, 1931  |
| Mannes et al.     | May 5, 1936   |
| Ostromislensky    | Aug. 17, 1937 |
| Lieber            | Aug. 16, 1938 |
| Knott             | Apr. 6, 1943  |
| Nadeau et al.     | Nov. 16, 1943 |
| Nadeau et al.     | May 30, 1944  |
| Ryan              | Oct. 22, 1946 |

## FOREIGN PATENTS

| Country       | Date          |
|---------------|---------------|
| Great Britain | Dec. 16, 1892 |
| Great Britain | Oct. 14, 1946 |